

March 3, 1959

H. SCHNEIDER

2,875,485

PRECISION CASTING MOLD AND METHOD OF MAKING THE SAME

Filed Dec. 14, 1954



Fig. 1

Fig. 5



Fig. 2



Fig. 3



Fig. 4



INVENTOR.

Hans Schneider

BY *James, Colombo, Monroe  
Borrome and Taylor*

ATTORNEYS

1

2,875,485

**PRECISION CASTING MOLD AND METHOD  
OF MAKING THE SAME**

Hans Schneider, Winterthur, Switzerland, assignor to Sulzer Freres, Societe Anonyme, Winterthur, Switzerland

Application December 14, 1954, Serial No. 475,244

Claims priority, application Switzerland  
December 17, 1953

4 Claims. (Cl. 22—193)

This invention relates to unitary precision casting molds and to a method of making the same. More particularly this invention relates to a unitary precision casting mold formed by means of a pattern destroyable in mold and in which the pattern is covered with a mold layer forming at least one thin non-self-supporting coating and which coating is backed-up with a dry, pourable backing up, or investment composition consisting of a mixture of a granular, refractory material and an inorganic bonding agent pulverulent at room temperature, and becoming an effective bonding agent at the temperatures used to bake the molds, and a dry pulverulent substance having a large active surface serving as a carrier for the inorganic bonding agent.

Prior processes, particularly where an intricate shape of a casting is to be made, do not come up to the imposed requirements. The backing up compositions used in these prior processes are unable to completely fill up recesses and back-sloping areas of the surfaces of the pattern coatings with the result that the pattern coatings are not adequately supported by the backing up compositions.

One known method for the production of unitary precision casting molds consists of forming a pattern of the casting, or several patterns thereof, from a fusible or combustible substance such as wax or a synthetic resin. The pattern is affixed to a sprue or pouring gate which serves as a positive pattern for the production of the casting mold. The sprue or pouring gate may also be formed from a fusible or combustible substance such as wax or a synthetic resin. The pattern and sprue are then coated with a fine refractory coating by immersing, or spraying them, in a liquid mixture of a very finely granular mold-forming substance, and a bonding agent to form a thin non-self-supporting coating over the pattern surface. The pattern is then dried out and is transferred into a molder's flask, and the cavity of the molder's flask filled with a backing up or investment substance consisting of a thickly fluid slurry of a granular molding compound to which a bonding agent has been added. The thin non-self-supporting coating limits the mold cavities and due to its finely granular constitution insures a smooth surface of the casting. The backing up compound provides a support for a non-self-supporting coating following the destruction of the pattern by the fusion or combustion of the pattern compound. The flowability of the thickly fluid backing up compound frequently causes defective castings. Such backing up compositions are unable to completely fill out the recesses and back-sloping areas of the non-self-supporting immersion coating with the result that these areas of the immersion coating are not sufficiently supported by the backing up compositions. The result of this is that during the casting operation, particularly in centrifugal casting practice, the molten metal breaks through the non-supported portions of the immersion coating. Furthermore the low flowability of the backing up composition limits the number of patterns that may be em-

2

bedded simultaneously in the single molder's flask since a large number of closely spaced patterns prevent the penetration of the backing up composition into the small interstices between the patterns. Furthermore, on baking the mold, the thickly fluid, highly viscous, backing up compositions become consolidated into a very hard ceramic body, thus rendering the extraction of the cooled casting from the mold a difficult and onerous operation. The utilization of any thickly fluid slurry backing up composition also calls for a very slow and careful drying out of the mold prior to baking it to prevent the formation of fissures and cracks.

According to the present invention a dry, pourable, backing up composition is used for supporting the thin non-self-supporting coating formed on the surface of the pattern. The dry, pourable backing up composition consists of a granular, refractory mold forming composition, and of an inorganic bonding agent pulverulent at room temperature, and a dry pulverulent substance serving as a carrier for the inorganic bonding agent and used for supporting the thin coating formed on the pattern surface. This composition has a substantially better flowability than a thickly fluid backing up composition and obviates to a far reaching extent the aforementioned disadvantages of prior processes when applied to precision casting molds. The backing up composition of the present invention is adapted to fill out uniformly even the smallest back-sloping areas and recesses, and provide an effective support for the thin non-self-supporting coating before and after the baking of the mold. Thus any break-through of the molten metal through the thin non-self-supporting mold layer which defines the pouring cavities may be effectively prevented and defective castings avoided.

The greater flowability of the dry backing up composition also enables one to pack a larger number of patterns into a single molder's flask at the same time. Drying out of the finished mold also becomes entirely superfluous, and the formation of fissures or cracks, such as that which occur when a thickly fluid backing up compound is dried, are prevented. The elimination of such a drying-out treatment and the withdrawal of the granular refractory material or sand from the cooled molder's flask likewise advantageously affect the economics of the casting process.

For a more detailed description of the invention, reference may be had to the accompanying drawing, in which:

Fig. 1 is a side elevation of a hollow cylindrical article with a flat bottom to be cast,

Fig. 2 is a schematic view of the destroyable pattern assembly,

Fig. 3 is a vertical section through a coated pattern assembly in a molder's flask,

Fig. 4 is a vertical section of the fired mold ready for casting, and

Fig. 5 is a top view of a hollow cylindrical article with a flat bottom to be cast.

Fig. 1 shows an article 10 to be cast which is a flat bottomed hollow cylindrical article. The wax patterns 11 are made of the article 10 according to the usual foundry practices taking into account the shrinkage of the metal to be cast. The wax patterns are made in suitable dies. In place of wax various thermoplastic resins, which may be destroyed in the mold, such as polystyrol, may be used. The wax patterns are cold-set and stripped from the dies, and assembled together conveniently for casting. The patterns are joined on to a wax feeder 13 by momentarily molding them at a point of contact with a heated instrument.

Fig. 2 shows a wax pattern assembly with patterns 11, ingate 12, and feeders 13. The ingates and feeders may also be composed of wax or a destroyable synthetic resin.

The pattern assembly as shown in Fig. 2 is ready for coating by immersing or spraying with a mixture consisting of a solid filler material and a suitable liquid binder. The binder serves to provide a close refractory film and the refractory filler material should have the property of forming a very smooth and refractory surface in contact with the wax pattern so that the cast article will be as smooth as possible.

The pattern assembly is then placed on a molding flask base plate 14 provided with a hole or perforation 15 as shown in Figs. 2 and 3. A cylindrical flask 16 is then fitted over the whole pattern assembly and the joint between base plate 14 and the flask 16 sealed with wax or by any other suitable sealing composition. A quick setting refractory mixture is then poured into the flask thus formed and permitted to stand until the mixture has sufficiently solidified to form a plate 19. Thereafter the dry, pourable, backing material is filled into the flask. The backing material consists of a refractory composition, a binder, or bonding agent, and a carrier for the bonding agent. The refractory material may consist of a granular material such as molding sand or quartz. The binding material is composed of a dry, finely ground powder at room temperature which becomes an effective bonding agent at the temperatures used to bake the mold. The carrier for the bonding agent is a pulverulent substance having a large active surface and which will readily absorb the inorganic bonding agent. Advantageously, the pulverulent carrier substance is impregnated with a solution of the bonding agent or with a fluid medium containing the bonding agent in a fairly finely divided solid form and subsequently dried. The dried pulverulent mass is then mixed with the refractory component of the investment composition. An advantage of using such a carrier for the bonding agent is that it brings a very large total surface area of the granular refractory molding compound into contact with the bonding agent adhering to the surface or pores of the pulverulent carrier. The pattern assembly provided with the thin non-self-supporting coating 17 is thus completely embedded in the backing material 18. The whole assembly is then placed on a vibration table, and vibrated sufficiently to insure that all surfaces of the coated pattern assembly are backed by the backing material. Thereafter a cover 20 is formed by pouring the same refractory mixture as used for the plate 19 on to the surface of the backing material.

In the next operation, the assembly shown in Fig. 3 is transferred into a furnace and fired by heating at a temperature of approximately 800-900° C. for 6-8 hours. This firing treatment causes the pattern material and the sprue material to melt. The wax or synthetic resin will partly flow out through the hole or perforation 15 or be burned. On baking the mold the bonding agent imparts a uniform cohesive strength to the investment. The investment compound having thus been consolidated has the property of protecting the thin mold layer effectively against destruction by the inflowing metal.

Fig. 4 shows the fired mold ready for casting. Molten metal is poured through the ingate 21 while the mold is still hot. The firing of the mold transforms the backing material into a refractory body 22 to which the coating 17 adheres.

Various granular, dry, refractory materials such as molding sands or quartz may be utilized as the refractory constituent of the backing composition without departing from the scope of the present invention.

The utilization of the dry pourable backing composition of the present invention entails a particularly careful bonding of the granular, refractory constituents of the backing up composition which on baking the mold imparts cohesive strength to the investment composition. Bonding agents suitable for the aforesaid purposes are those inorganic compounds which bring about a bonding action during the baking of the mold and which have

a high adhesivity or a great capacity of sticking to the granular refractory compound of the backing up composition. Particularly suitable are gel-like inorganic compounds pulverulent at room temperature and which become fusible at temperatures above 600° C. and preferable between 800 and 1000° C. The backing up composition, having been bonded, is adapted to protect the thin mold layer reliably against destruction by the inflowing molten metal.

Some examples of suitable inorganic bonding compounds are liquid dispersions of gelatinous bonding agents such as complex aluminium pyrophosphates, alkali-metal zirconates, alkali-metal titanates, titanic acids, zirconic acids, or oxychlorides such as magnesium oxychlorides. These compounds are distinguished in that at room temperature they exhibit a gel-like structure in a dry condition. Other examples are solutions of borates, such as borax dissolved in water, phosphoric acid and boric acid. Solutions of phosphates such as primary sodium phosphate may also be used.

Various carriers for the inorganic bonding agents may be used in accordance with the present invention. Some examples of carriers which have large active surfaces and exhibit a high adhesivity or capacity of absorbing the inorganic bonding agents due to their porous constitution and their highly particulate surface are infusorial earth, magnesium silicates such as meerschaum, pumice, and asbestos. Other substances have a large active surface and the above properties may also be used as a carrier in accordance with the present invention. The above named compositions, however have been found to be particularly advantageous in the present invention.

When larger size patterns are to be invested or backed it is also advantageous to admix with the backing up composition comprising a dry, pulverulent, refractory material, an inorganic bonding agent effective at temperatures above 600° C. and a carrier for the inorganic bonding agent, a second bonding agent dry at room temperature and becoming an effective bonding agent at temperatures below the baking temperatures of the mold, or below 600° C. Examples of such bonding agents are finely ground synthetic resins, such as silicone resins, which become an effective bonding agent at a moderately high temperature. This second bonding agent may be used when the rigidity of the raw unbaked molds do not resist the vibrations occurring during their transportation.

#### Example

A plurality of wax patterns of a small flat bottomed hollow cylindrical article were assembled together with a sprue in the form of a tree-like structure which serve as a positive pattern for the production of the casting mold. The sprue was similarly made of wax. The composite tree-like pattern thus constructed was then dipped into a liquid mold forming composition of a mixture prepared from finely comminuted quartz and partly hydrolyzed ethyl silicate dissolved in alcohol as is well known in the art. The thin non-self-supporting film deposited on the pattern was about 0.5-1 mm. in thickness. This coating was then dried and the pattern placed with the sprue downward upon a plate perforated for the subsequent discharge of the molten wax pattern. A cylindrical molder's flask made of heat-resisting sheet metal was then placed over the entire coated pattern and the joint between the flask and the perforated plate was then sealed off with wax. A small amount of a liquid mixture of quartz sand and water glass to which an acid, such as hydrochloric acid, had been added for the purpose of accelerating the hydrolysis, was then added to the flask. This fluid mixture was permitted to stand until solidified to form a cover plate surrounding the sprue. The molder's flask was then filled up with a dry, pourable backing up composition which was prepared as follows: 600 grams of primary sodium phosphate was dissolved in 2

liters of water and the solution added to 2.4 kg. of comminuted infusorial earth. Infusorial earth consists of the minute fragments of the shells of silicious algae (diatomae). It is characterized by a very large active surface. The mixture of primary sodium phosphate and infusorial earth was thoroughly kneaded and dried overnight at about 120° C. The dried composition was then ground and particles above 40 microns removed therefrom by means of a fine mesh screen. 6 parts by weight of the pulverulent substance thus obtained were mixed with 94 parts by weight of quartz sand having a particle size between 0.5 and 1.0 mm., and the whole thoroughly commingled in a rotary drum. This dry, pourable backing up composition thus obtained, containing an inorganic bonding agent, was packed into the molder's flask and firmly settled therein on a shaking table. The top face of the molder's flask was then covered with a slurry-like mixture of quartz sand and water glass, to which an acid had been added to accelerate the hydrolysis, to form a second cover plate the same as that formed above. After the cover had hardened the molder's flask was transferred into a baking furnace and gradually raised to a baking temperature of 800° C. during a period of 6-8 hours. During the baking operation the sodium phosphate deposited upon the infusorial earth fuses and in that state exerts the desired bonding action on the investment composition. If the wax pattern is to be recovered, the mold prior to being baked, is transferred into a drying oven in which the wax is caused to run out at a slightly raised temperature. Immediately upon removal of the molder's flask from the baking furnace, liquid metal was poured in the mold. After cooling the mold, the two covers were broken up and the waste mold forming composition knocked out of the molder's flask. The castings may be readily taken out of the backing up composition 35 and freed from any mold forming composition still adhering thereto in any conventional manner. The finished castings exhibited a perfectly smooth surface free from blemishes and form a particularly true replica of the pattern parts.

In case of larger size molds, it is advantageous to use armoring members for the purpose of strengthening the investment compound. Casting molds produced in accordance with the process of the invention are adapted for static castings as well as for making castings on a 45 centrifugal casting machine.

I claim:

1. The method of making a unitary precision casting mold by means of a pattern destroyable in the mold which comprises coating the pattern with at least one 50 mold forming layer having the form of a thin non-self-supporting coating, placing the pattern in a molder's flask, backing up the coated pattern with an investment composition comprising a dry pourable composition containing a granular, refractory, molding composition, an inorganic bonding agent, and a carrier which is a member selected from the group consisting of infusorial earth, magnesium silicate, meerschaum, pumice, and asbestos impregnated with the bonding agent comprising a dry,

5 pulverulent composition having a large active and porous surface and a high capacity for absorbing inorganic bonding agents, the particle size of said refractory composition being substantially larger than the particle size of said impregnated carrier, and heating the mold to the baking temperature of the mold to destroy the mold pattern and to permit adherence of the pattern coating to the backing up composition, said carrier impregnated with said inorganic bonding agent being dry and pulverulent at room temperature and said bonding agent becoming an effective bonding agent at the temperature used to bake the mold.

2. The method of claim 1 in which the carrier is impregnated with a composition selected from a member of the group consisting of phosphates, phosphoric acid, borates, boric acid, complex aluminium pyrophosphates, zirconic acid, alkali-metal zirconates, titanic acid, and alkali-metal titanates.

3. An investment back up composition for unitary precision casting molds in which the mold pattern is defined by at least one mold forming layer in the form of a thin non-self-supporting coating and in which the molds are formed by baking the coated pattern and back up composition comprising a dry, pulverulent, pourable composition containing a granular, refractory, molding composition and a carrier which is a member selected from the group consisting of infusorial earth, magnesium silicate, meerschaum, pumice, and asbestos impregnated with an inorganic bonding agent, said carrier comprising a dry, pulverulent composition having a large active and porous surface and a high capacity for absorbing inorganic bonding agents, and said bonding agent being dry and pulverulent at room temperatures and becoming an effective bonding agent at the temperature used to bake the mold, said back up composition comprising between about 85 to 96 parts by weight of refractory material, between about 3 to 10 parts by weight carrier, and between about 1 to 5 parts by weight of inorganic binder on a dry basis.

4. The investment, back up composition of claim 3 in which the carrier composition is impregnated with a composition selected from the group consisting of phosphates, borates, phosphoric acid, complex aluminium pyrophosphates, zirconic acid, alkali-metal zirconates, titanic acid, and alkali-metal titanates.

#### References Cited in the file of this patent

#### UNITED STATES PATENTS

|           |               |               |
|-----------|---------------|---------------|
| 2,027,932 | Ray           | Jan. 14, 1936 |
| 2,388,299 | Thielemann    | Nov. 6, 1945  |
| 2,441,695 | Feagin et al. | May 18, 1948  |
| 2,521,614 | Valyi         | Sept. 5, 1950 |
| 2,682,692 | Kohl          | July 6, 1954  |
| 2,720,687 | Shaw          | Oct. 18, 1955 |
| 2,736,077 | Bartlett      | Feb. 28, 1956 |

#### FOREIGN PATENTS

|         |               |               |
|---------|---------------|---------------|
| 585,665 | Great Britain | Feb. 18, 1947 |
| 703,607 | Great Britain | Feb. 3, 1954  |